

# UNITED STATES PATENT OFFICE.

WILLIAM EDGAR MUNTZ, OF LONDON, ENGLAND.

## TREATMENT OF FIBERS TO INCREASE THEIR COEFFICIENT OF FRICTION ON EACH OTHER.

1,232,374.

Specification of Letters Patent.

Patented July 3, 1917.

No Drawing.

Application filed April 4, 1914. Serial No. 829,553.

*To all whom it may concern:*

Be it known that I, WILLIAM EDGAR MUNTZ, a subject of the King of Great Britain, and resident of 6 Bream's Buildings, Chancery Lane, London, England, late of His Majesty's Public Works Department, India, have invented new and useful Improvements in the Treatment of Fibers to Increase Their Coefficient of Friction on Each Other, of which the following is a specification.

There are many fibers which have hitherto defied the efforts of the spinner to spin them into a satisfactory yarn.

15 These are fibers of a smooth and slippery nature with little or no tendency to cling together. These, particularly if deficient in length, either cannot at present be spun at all, or if spun make a yarn so weak as to be 20 useless or nearly so for practical purposes.

I now propose to render such fibers useful by treating them to make them less susceptible to slipping over each other so that they will assume a capacity for cohesion.

According to my invention the fibers are completely and evenly covered all over with an extremely thin coating of material possessing a higher coefficient of friction.

The coating which I employ is contained 25 in a mobile solution which may be dried off or evaporated leaving the coating behind on the fibers.

This solution must be mobile and completely fluid at the time of its application 35 and free from all trace of viscosity or lumpiness so as to freely penetrate between and around the fibers, and evenly spread itself over them, pressure or vacuum being employed when required to expel air bubbles 40 and thereby insuring the deposit of an even excessively thin coating all over the fibers.

I am aware that it has been proposed to manufacture yarns, threads, and fabrics of certain smooth fibers by twisting the fibers 45 into rovings by two successive workings on rota condensers either wet or dry, also that seed hairs of kapok and the like have been treated with solvents adapted to withdraw therefrom incrusting substances whereby the 50 said hairs are caused to shrink and acquire a rough surface.

I am also aware that it is a common practice to spin brittle or slippery fibers around a matrix or core or intertwined with rougher 55 and stronger fibers. Another practice is to

agglutinate the fibers to form coarse threads to be afterward cased and woven or to agglutinate the fibers into a lap or sheet to be afterward cut into strips for use in spinning and weaving.

As far as I am aware however no attempt has ever yet been made to cover the fibers individually, completely, and evenly all over before the spinning is completed with an extremely thin coating of material which material shall have a higher coefficient of friction than the surface of the fibers, so that the fibers thus coated shall have a greater resistance (by friction under pressure due to twist, weight, etc.) to slip over each other, without their drawing action necessary for spinning being seriously affected.

The treatment may be imparted to the fiber when in an entirely loose condition or, if the fibers are capable of being spun sufficiently to permit of handling, the treatment may preferably be deferred until such preliminary spinning or twisting has been effected.

The treatment which I propose will consist in depositing on the surface of the fibers a substance which will adhere thereto without prejudicially affecting the fibers or the substances to come in contact with them and will, at the same time, roughen the slippery surface of the fibers to prevent more than the amount of slipping over each other than is necessary in the "drawing out" incidental to spinning, the excessive slipping having hitherto baffled the efforts of the spinner.

The treatment would have the incidental advantages, viz:—(1) that short light fibers would cohere during spinning and "flying" would be obviated; (2) that any adhering action after spinning would be along the whole length of the fiber, so that the adhering surfaces would not tear apart (give) before fracture of the fiber itself; (3) completely covering fibers would act as protection from damp, acid, etc., and other influences deleterious to strength of fiber.

If the fiber were not evenly covered, it would militate against the "drawing out" incidental to spinning and, more important, the adhesion between the fibers would be interrupted and therefore of less sectional area and consequently less effective against fibers slipping prior to their fracture.

To take an example in connection with "undischarged" waste silk, (by which I

60

65

70

75

80

85

90

95

100

105

110

mean the refuse of cocoons in which fibers still retain their natural gum). Ordinarily, many of these fibers are more or less short and if spun with the gum in, during 5 spinning these short fibers "fly" apart and also have not a sufficiently large coefficient of friction to enable them to be easily spun, or even if this can be done, to prevent their slipping over one another when once spun 10 before they fracture when yarn is subjected to strain.

In dealing with waste silk, still containing 15 its natural gum, (which for various reasons it is often desirable to retain,) after washing in petrol or the like, I immerse the fibers under pressure or vacuum if necessary, in a dilute solution of india rubber or other roughening material of such a strength that while such solution is sufficiently mobile to 20 penetrate between and around the fibers, it is yet strong enough to cause the deposition all over the fibers of only a sufficient thickness of rubber adhering to these fibers to prevent undue slipping over each other 25 both during spinning and also in the yarn. The solvent, which shall be volatile, is evaporated, (preferably in a closed chamber with a view to recovery) leaving the fibers roughened and more susceptible of 30 advantageous spinning into yarn. If fibers adhere during treatment before spinning re-carding will be necessary after treatment unless spun wet.

Many substances other than "waste" silk 35 can be so treated with advantage, and some hitherto incapable of spinning can thus be made into yarn. Probably in most cases the greater advantage will be got by treating the yarn after loosely spinning and then 40 drying in a more twisted state, in order to reap the full benefit of the cementing action and avoid the uncovering of the fiber by possibly re-carding necessary immediately before spinning. The fibers cannot 45 be left cemented together before spinning, otherwise "drawing out" would be prevented.

It will probably be possible to spin this-tideworn, deep-sea fiber (*Posidonia Australis*) and other fibers which have hitherto defied human ingenuity, and many other short and slippery fibers would be enormously strengthened in the yarn.

The liquid used in the treatment may 55 comprise, a dilute mobile solution of rubber in carbon bisulfid, benzol or other suitable solvent, or a dilute mobile solution of gelatin in water or other suitable solvent in any form, or similar substances. To these 60 solutions may or may not be added glycerol or other hygroscopic or other substance in sufficient quantity to keep the coating of rubber, gelatin, or similar material in a "tacky" state. Also the deposit of rubber 65 might subsequently be hardened by vul-

canization, the sulfur chlorid, sulfur or other material required for vulcanization being (1) either incorporated in the original solution used in the treatment, or (2) introduced into the fibers, yarn, or fabric 70 after the coating treatment, or (3) derived from suitable rubber mixtures coated on to the yarn or fabric subsequently, and the fibers, yarn, or fabric subjected if desired to any heat required for vulcanization at 75 any convenient stage in the process of manufacture subsequently to treatment with the rubber solution or after use of yarn in weaving or otherwise or during the vulcanization of any rubber mixture that might be 80 coated on to the yarn or fabric. Further, the deposit of gelatin, isinglass, or similar material, with or without glycerin left on the fibers (whether or not worked up into yarn or fabric or whether or not such yarn 85 or fabric has been woven, knitted, netted, or otherwise used) by the evaporation of the solvent or removal of the re-agent or influence rendering it sufficiently mobile to completely and evenly cover the fibers all 90 over may preferably be subsequently hardened and rendered absolutely insoluble in water by treatment with formalin (formaldehyde), alum, chrome-alum, potassium bichromate, or other agent having a like effect. Or again, the fiber or yarn may be treated with a solution of gum-arabic or 95 other suitable gum with or without glycerin, and dried, and the deposit subsequently hardened and rendered completely insoluble 100 in water (whether before spinning or weaving or whether yarn or fabric has been used or not) by treatment with a solution of potassium bichromate or other reagent having a similar effect. The hardening process 105 should in most cases, but especially when potassium bichromate or chrome alum is used be carried out with free exposure of the fibers to light, as it is well known that light facilitates the hardening action of 110 certain reagents.

Other liquids or solutions which could be employed are glycerin, alone, or preferably diluted with water or otherwise to render it mobile (which could, if desired, be 115 afterward removed from the spun yarn or woven fabric by washing with water) or a dilute mobile solution of animal glue or gelatin in acetic acid prepared in a manner that is well understood so as to be insoluble in water after it has once been dried.

To the solution employed may sometimes be added if desired a suitable solid material in a fine state of division held in suspension which will remain adhering to the fiber after 120 solvent is evaporated.

The following are examples of working with waste silk:—

Example 1: Silk waste "undischarged" after cleaning with petrol or other agent 130

which will not touch the gum or damage the silk, is immersed, preferably under pressure or in vacuum, in a 5% solution of rubber dissolved in pure carbon bisulfid (of boiling point not lower than 46° centigrade) and allowed to remain under conditions favorable to evaporation and recovery of solvent until solid matter alone remains on the fiber, the solvent entirely separating itself by evaporation. (1) Finely divided rough particles may be added to solution or (2) these particles may while suspended in air be dusted on or breathed through the silk fibers while rubber coating is still "tacky" or (3) particles may be rubber coated, then mixed with fibers and cemented to them by immersing whole mass in vapor of solvent.

Example 2: Yarn loosely spun from "undischarged" silk "waste" is cleaned with petrol or other agent which will not touch the gum or damage the silk, and is immersed, preferably under pressure or in vacuum, in a 5% solution of rubber dissolved in pure carbon bisulfid (of boiling point not lower than 46° centigrade) or dissolved in benzol or naphtha for 10 minutes, twisted as it comes from the solution before evaporation of solvent, wound on a bobbin, and allowed to remain under conditions favorable to evaporation and recovery of solvent until solid matter alone remains on the fiber, the solvent entirely separating itself by evaporation.

If the liquid or solution which has been used to render the fibers less susceptible to slipping on each other contains a substance which would subsequently prove useless, disadvantageous or injurious, such as gelatinous rubber, resinous, or other similar substances, this substance may be extracted from the fibers by a solvent or by a mechanical process applied at that stage in the manufacture which appears to be most appropriate and the most convenient for this operation.

What I claim and desire to secure by Letters Patent in the United States is:—

1. The process of manufacturing yarn

from fibers which are too slippery to be successfully spun when in their normal condition, consisting in treating the fibers before the spinning is completed with a solution mobile and completely fluid at the time of its application and thereby depositing an adhering coating on the fibers which shall increase the coefficient of friction of the fibers over one another to render the complete spinning of the fibers into yarn feasible and without seriously affecting the drawing out action incidental to the spinning.

2. The process of manufacturing yarn from fibers which are too slippery to be successfully spun when in their normal condition, consisting in treating the fibers before spinning with a solution mobile and completely fluid at the time of its application and thereby depositing an adhering coating on the fibers which shall increase the coefficient of friction of the fibers over one another to render the complete spinning of the fibers into yarn feasible and without seriously affecting the drawing out action incidental to the spinning.

3. The process of manufacturing yarn from fibers which are too slippery to be successfully spun when in their normal condition, consisting in treating the fibers before the spinning is completed with a mobile solution of rubber and completely fluid at the time of its application and thereby depositing an adhering coating on the fibers which shall increase the coefficient of friction of the fibers over one another to render the complete spinning of the fibers into yarn feasible and without seriously affecting the drawing out action incidental to the spinning and subsequently hardening said friction coating for the purposes substantially as set forth.

In testimony whereof I have signed my name to this specification in the presence of two subscribing witnesses.

WILLIAM EDGAR MUNTZ.

Witnesses:

L. A. NEWTON,  
E. C. WALKER.